

April 14, 1931.

W. E. RUDER

1,801,110

METHOD FOR WORKING NORMALLY BRITTLE SHEET METAL

Filed May 8, 1928



Inventor:  
William E. Ruder,  
by *Charles E. Tullar*  
His Attorney.

## UNITED STATES PATENT OFFICE

WILLIAM E. RUDER, OF SCHENECTADY, NEW YORK, ASSIGNOR TO GENERAL ELECTRIC COMPANY, A CORPORATION OF NEW YORK

## METHOD FOR WORKING NORMALLY-BRITTLE SHEET METAL

Application filed May 8, 1928. Serial No. 276,175.

The present invention relates to a method for working normally brittle sheet metal, and more particularly to a method for treating an iron base resistance alloy containing appreciable amounts of chromium and aluminum.

In my copending application, Serial No. 147,388, filed November 9, 1926, there is disclosed a resistance alloy of this type having an iron base and containing a small amount of an element of the third horizontal group of Mendeleff's periodic table, such as aluminum and a larger amount of chromium. A small amount of carbon preferably less than one tenth per cent and less than one per cent each of silicon and manganese may be present in the alloy. The alloy usually contains the above metals in the following percentages by weight:

|    |           |               |
|----|-----------|---------------|
| 20 | Aluminum  | 4-6%          |
|    | Chromium  | 12-15%        |
|    | Carbon    | less than 10% |
|    | Silicon   | less than 1%  |
| 25 | Manganese | less than 1%  |
|    | Iron      | remainder     |

These proportions may be varied somewhat depending upon the properties desired in the alloy. For example, the aluminum content may be as low as 2% and the chromium content as low as 10%.

The alloy containing the above ingredients has very desirable mechanical and electrical properties and in addition is comparatively inexpensive. These qualifications render it particularly suitable for use as a resistor element in control rheostats. In manufacturing such rheostats the alloy is rolled into thin flat strips which are subjected to a shearing operation to produce a narrow thin metal ribbon which is wound edgewise into a coil to provide the resistor element of the rheostat. The shearing operation apparently produces a certain degree of brittleness in the material, so that when wound into a coil having substantially rectangular form considerable difficulty has been encountered due to the tendency of the material to break or fracture at the points where it is bent sharply at right angles to

itself. It is one of the objects of the present invention to provide means whereby this difficulty may be avoided.

The novel features which I believe to be characteristic of the invention are set forth with particularity in the appended claims. The invention itself however will best be understood from reference to the following specification when considered in connection with the accompanying drawing in which the single figure shows diagrammatically a perspective view of an apparatus whereby the invention may be carried into effect.

Referring more particularly to the drawing, I have indicated at 1 a bending machine comprising a hardened steel bending die 2 which is carried by a solid steel wheel 3, the latter being driven from a source of power through a pulley 4 and belt 5. The alloy conductor comprises a relatively thin flat ribbon 6 which may be wound upon a wheel 7 and fed to the die 2 through an electrical heating coil 8 supplied from a source of energy not shown. The wheel 3 and die 2 are heated by a plurality of blow torches 9 or any other suitable means.

Coil 8 and blow torches 9 warm the alloy conductor 6 and die 2 to a temperature which is well below 200° C. but at which the conductor may be bent without danger of fracture. I have found that a temperature above 80° and in the neighborhood of 100° C. will give uniformly satisfactory results. While the temperature may vary considerably, it should be well above room temperature and well below 200° C. The latter temperature should not be exceeded, since the hardened steel bending die will become progressively softened about this temperature and soon become useless.

After the process has been in operation for some time the heat supplied by coil 8 may be increased slightly and the heating of the wheel 3 and die 2 by means of blow torches discontinued. It will be found that the heat supplied by the coil 8 after the process has been in operation for some time is sufficient to keep the die 2 warm enough so that the ribbon conductor may be bent into the desired form

without causing any break or fracture in the material.

What I claim as new and desire to secure by Letters Patent of the United States is:

- 5 1. The method of winding a flat metallic conductor edgewise into a coil, which comprises heating the conductor to a temperature well above room temperature and well below 200° C. and then winding it on a die warmed to approximately the same temperature as the conductor.
- 10 2. The method of winding a flat normally brittle electrical conductor edgewise into a coil, which comprises heating the conductor 15 and winding it on a heated die, the temperature of the conductor and die being below 200° C. but high enough to prevent fracture of the material when bent into a rectangular-shaped coil.
- 20 3. The method of producing sharp bends in sheet metal which consists largely of iron but contains appreciable amounts of chromium and aluminum, which comprises heating the metal to a temperature above room temperature and well below 200° C. and then bending 25 it on a die having approximately the same temperature as the conductor.
- 30 4. The method of making resistance grids from strip material composed of an iron-chromium-aluminum alloy in which the chromium content ranges from about 10% to about 15%, the aluminum content from about 2% to about 6% with the remainder iron except for incidental impurities, which consists 35 in heating the strip to a temperature well above room temperature but below 200° C., and then bending it edgewise on a die warmed to a temperature below 200° C. but well above room temperature.
- 40 40. In witness whereof, I have hereunto set my hand this 7th day of May, 1928.

WILLIAM E. RUDER.